

# UNITED STATES PATENT OFFICE.

EZECHIEL WEINTRAUB, OF NEW YORK, N. Y., ASSIGNOR TO GENERAL ELECTRIC COMPANY, A CORPORATION OF NEW YORK.

## CATALYZING MATERIAL.

1,299,641.

Specification of Letters Patent. Patented Apr. 8, 1919.

No Drawing.

Application filed March 26, 1918. Serial No. 224,895.

To all whom it may concern:

Be it known that I, EZECHIEL WEINTRAUB, a citizen of the United States, residing at New York, in the county of New York, State 5 of New York, have invented certain new and useful Improvements in Catalyzing Material, of which the following is a specification.

The present invention comprises a new 10 form of catalyzer, consisting of a catalyzing agent and a support, which is peculiarly adapted to produce a higher speed of reaction than formerly attainable.

Heretofore catalyzing metals such, for example, as platinum and nickel have been deposited either on granular material or on a fibrous material such as asbestos.

I have discovered the peculiar adaptability as a catalytic support of an artificial material known as fibrox described by me in *Transactions of the American Electrochemical Society*, Vol. XXVII, (1915) p. 267, and also in Patent #1,094,352, of April 21, 1914. Fibrox is a soft, compressible material, consisting of a mass of fine interlacing fibers, the mass being usually greenish or white in color and having an apparent density of about 0.0070 to 0.0025.

The speed of reactions facilitated by catalyzers is proportional to the surface exposed by the catalyzer. The fibers of fibrox are not only very fine, the diameter of the fibers on the average being only about 0.0006 inch, or about the wave length of yellow light, but which is even of greater importance in this combination, the fibers, unlike asbestos, are originally formed separated from each other by relatively large spaces or voids. These two factors give fibrox an enormous surface per unit volume so that when a mass of fibrox having its fibers coated with a catalyzer, is traversed by gases, the effective catalyzer surface in contact with the gases is of a different order 45 of magnitude than in any other known catalytic support, granular or fibrous. The fibers of fibrox are also adapted to catalytic reactions because they withstand high temperatures, are inert to most of the gases and 50 are resilient and self-supporting. Oxidizing gases like oxygen will at elevated temperatures transform the silicon oxycarbide of which the fibers consist, into silica but as this transformation is not accompanied by

change of structure the effectiveness of the 55 material as a catalytic support is not impaired when thus oxidized. Such transformation products of the described material which have the essential physical structure of fibrox are also to be included under 60 the same generic name of "fibrox".

The new catalyst comprising my invention may be prepared by either of the following methods which may, of course, be in turn modified in various respects:

*Deposition from gaseous mixtures.*—According to one method, finely divided metal is deposited on the surface of fibrox fibers by the reduction of a vapor compound of the respective metal in contact with the 70 fibers. For example, finely divided nickel may be deposited by the decomposition of nickel carbonyl vapor in contact with fibrox, platinum may be deposited on the fibrox by the reduction of carbonyl platino-chlorid 75 and osmium deposition may be carried out by the reduction of vapors of osmium tetrachlorid with hydrogen.

Fibrox strips may be placed in a container of glass, quartz or the like. The air 80 may be preferably withdrawn with a vacuum pump and the vapor of nickel carbonyl then is admitted preferably at reduced pressure, say at about one-fifth atmosphere, 85 in order to allow for the increase in volume and pressure when the carbonyl decomposes. The container when thus charged is heated to about 180° C. in order to decompose the nickel carbonyl, depositing finely divided nickel on the fibrox fibers. This treatment may be repeated several times to produce a desired deposit.

When a deposit of platinum is desired, the fibrox is placed in a container of glass, quartz or other material sufficiently refractory and a quantity of carbonyl platino-chlorid is admitted. This material may be formed in a chamber immediately adjacent the fibrox container by the action of carbon monoxid and chlorin gas on platinum 100 sponge at a temperature of about 250° C. The platinum is deposited by heating as above described in connection with the deposition of nickel.

*Deposition from solutions.*—When it is 105 desired to deposit a coating of nickel upon the fibrox fibers by the solution process, nickel sulfate is dissolved in water and to

the solution about twice the amount of sodium hypophosphite is added which is theoretically required to reduce the nickel sulfate. The fibrox is immersed in this 5 solution and the solution is heated to boiling. The resulting chemical action involves the formation of nickel hypophosphite and its subsequent reduction on continuous boiling by the excess of sodium hypophosphite 10 to form metallic nickel. The boiling is continued for at least an hour and thereupon the fibrox is removed, carefully washed with distilled water, and finally dried. If the washing operation with distilled water has 15 been thoroughly done so as to leave no un-reduced salts upon the fibrox, then the coated fibrox will return to its initial bulk upon drying.

Similarly a mass of fibrox may be placed 20 in a solution of chlorplatinic acid and an excess of saturated solution of ferrous sulfate is added and the solution mixture is boiled. The result is a deposition of platinum on the fibers of the fibrox which 25 thereupon should be thoroughly washed with distilled water.

The fibrox catalyst may be used for the

oxidation of ammonia to nitric acid, the oxidation of sulfur dioxide to form sulfur trioxide for the manufacture of sulfuric acid, 30 and particularly for the synthesis of ammonia from nitrogen and hydrogen. In this case as high pressure is used a small sized apparatus is desirable and therefore the large active surface offered by fibrox for 35 a small volume is of special advantage.

In my copending application, Serial No. 224,897, filed concurrently herewith, claims have been made on a process of preparing the catalyst described herein. 40

What I claim as new and desire to secure by Letters Patent of the United States, is:

1. A catalyst comprising fibrox and a deposit of catalyzing material on the fibers thereof. 45
2. A catalyst comprising a mass of interlacing fibers of silicon oxy-carbide, spatially separated from each other and a deposit of catalyzing material on said fibers.
3. A catalyst comprising fibrox and a deposit of nickel on the fibers thereof. 50

In witness whereof, I have hereunto set my hand this 20th day of March, 1918.

EZECHIEL WEINTRAUB.